

## UNITED STATES PATENT OFFICE

2,402,437

## LACQUER

Herbert Stuart Northway, Helsby, near Warrington, England, assignor to British Insulated Cables Limited, Prescot, Lancashire, England, a British company

No Drawing. Application December 8, 1944, Serial No. 567,328. In Great Britain January 22, 1944

1 Claim. (Cl. 106—171)

1

This invention relates to lacquers and is more particularly concerned with the production of a lacquer that is suitable for application to insulated electric wires and cables. For such purposes it is desirable that the lacquer should yield a lacquer film that maintains its flexibility over a wide temperature range, for instance, a range extending from  $-20^{\circ}\text{ C.}$  to  $150^{\circ}\text{ C.}$  The lacquer film should be both hard and tough and should not fuse to adjacent lacquer films under high operating temperatures. It should also be resistant to hot oil, petrol and water and should have a low co-efficient of friction that will permit a lacquer coated insulated wire or cable to slide easily over similar wires or cables with which it is in contact. It is the object of my invention to produce an improved lacquer that will yield lacquer films possessing the aforesaid characteristics to a high degree.

In accordance with the invention my improved lacquer comprises a solution containing ethyl cellulose having an ethoxy content of from 43.5% to 46.5% and a viscosity of from 100 to 250 centipoises, and from 2 to 4 parts by weight of transformer oil, from 2 to 4 parts by weight of petroleum jelly and from 3 to 6 parts by weight of castor oil, to each 10 parts by weight of ethyl cellulose.

By "ethoxy content" is meant the weight of ethoxy radical ( $\text{OC}_2\text{H}_5$ ) expressed as a percentage of the ethyl cellulose molecule. As is known, this percentage may vary from a value approaching zero to a value approaching 55%, corresponding to an average value of from nearly 0 to 3 ethyl radicals per glucose unit. The selected range which I employ with the specified proportions of particular plasticisers in order to obtain my improved heat-resistant lacquers is comparatively narrow, being from 43.5% to 46.5%, corresponding to an average value of 2.15 to 2.35 ethyl radicals per glucose unit.

As a solvent for the ethyl cellulose and the plasticisers I prefer a mixture of benzene and alcohol (methylated spirit) in which the benzene predominates, the optimum proportion of benzene to alcohol being of the order of 2 to 1. If desired acetone may be substituted for a part of the benzene, but this will entail a slight increase in the viscosity of the lacquer.

2

Examples of compositions of my improved lacquers are given in Table I below:

Table I

|    |                                                                            | I    | II   | III  | IV   |
|----|----------------------------------------------------------------------------|------|------|------|------|
|    | Ethyl cellulose having ethoxy content of 45-46.5% and viscosity of 150 cps |      |      |      |      |
|    | .....grams.....                                                            | 10.0 | 10.0 | 10.0 | 10.0 |
| 10 | Castor oil (raw or bodied).....do.....                                     | 4.0  | 6.0  | 4.5  | 5.0  |
|    | Transformer oil.....do.....                                                | 2.0  | 2.0  | 2.2  | 2.2  |
|    | Petroleum jelly.....do.....                                                | 2.0  | 2.0  | 2.2  | 2.3  |
|    | Benzene.....cubic centimeters.....                                         | 42   | 42   | 42   | 42   |
|    | Alcohol (methylated spirit).....do.....                                    | 18   | 18   | 18   | 18   |

If desired my improved lacquer may incorporate a spirit-soluble dye. The amount of dye used is of the order of 0.5% by weight on the ethyl cellulose content of the lacquer. Conveniently it is added as a 1% solution in alcohol, in which case the proportion to be used with each of the compositions specified in Table I above is 5 ccs.

The high quality of the lacquer films obtained from these lacquer compositions will be gathered from Table II below, which gives results of numerous tests carried out on films obtained from the lacquers given in Table I, and for purposes of comparison, from a lacquer, designated V, which prior to my invention has been regarded as the most satisfactory for the purpose in view.

Table II

|    | Test on film                                                      | I     | II    | III   | IV    | V      |
|----|-------------------------------------------------------------------|-------|-------|-------|-------|--------|
| 35 | Tensile strength.....lbs. per sq. in.                             | 2,050 | 2,475 | 2,650 | 2,450 | 1,050  |
|    | Percentage elongation at break.....                               | 55    | 75    | 55    | 70    | 60     |
|    | Product of tensile strength and elongation $\times 10^{-4}$ ..... | 11.2  | 18.6  | 14.6  | 17.2  | 6.3    |
|    | Shore hardness at $20^{\circ}\text{ C.}$ .....                    | 95-93 | 88-86 | 95-93 | 93-90 | 87-85  |
|    | Shore hardness at $150^{\circ}\text{ C.}$ .....                   | 45    | 20    | 45    | 42    | 45     |
| 40 | Flow test.....pounds.....                                         | 0.25  | 0.2   | 0.3   | 0.2   | 0.2    |
|    | Friction test.....do.....                                         | 1.0   | 1.5   | 1.5   | 1.5   | Over 6 |

The Shore hardness at  $20^{\circ}\text{ C.}$  was measured, applying the durometer by hand, initially and after 30 seconds application. The flow test consisted in pressing together two films under a pressure of 1 lb. per square inch for two hours at  $150^{\circ}\text{ C.}$  and in measuring the weight necessary to separate the films after cooling to room temperature for one hour. The value recorded is in pounds per one inch width of film. The fric-

tional properties of the film were assessed by fixing it to a cylindrical metal disc having a diameter of 2.5 inches and a thickness of 0.5 inch placing the film covered disc on to another film of lacquer so that the two films were in contact, and measuring the horizontally applied force in pounds required just to keep the one film sliding over the other when a 7 lb. weight had been placed on the disc.

Tests on the heat resisting cores of 7 mms. diameter lacquered with my improved lacquer showed the lacquer to be very flexible at normal temperatures and to possess ample flexibility at temperatures as low as  $-35^{\circ}$  C., and also after being heated for 100 hours at a temperature of 15

$150^{\circ}$  C. Tests on such cores also showed that coatings of adjacent cores were easily separated from one another when cooled after being heated in contact for a period of two hours at  $150^{\circ}$  C.

5 What I claim as my invention is:

A lacquer comprising a solution containing ethyl cellulose having an ethoxy content of from 43.5% to 46.5% and a viscosity of from 100 to 250 centipoises, and to each ten parts by weight of ethyl cellulose, from 2 to 4 parts by weight of transformer oil, from 2 to 4 parts by weight of petroleum jelly and from 3 to 6 parts by weight of castor oil.

10 HERBERT STUART NORTHWAY.